

Patented Jan. 31, 1928.

1,657,982

# UNITED STATES PATENT OFFICE.

WARREN WILKIE AND ALEXANDER D. WEBB, OF DETROIT, MICHIGAN, ASSIGNEES TO PARKE, DAVIS & COMPANY, OF DETROIT, MICHIGAN, A CORPORATION OF MICHIGAN.

## PROCESS OF MANUFACTURING GELATIN CAPSULES FOR USE AS BOTTLE CAPS.

No Drawing.

Application filed February 15, 1926. Serial No. 88,503.

This invention relates to a process of manufacturing gelatin capsules for use as bottle caps, and has as its principal object to treat the caps during the process of manufacture, so as to raise the melting point of the gelatin to thereby eliminate the characteristic stickiness of unmodified gelatin, and to render the caps immune to changes in temperature and climatic conditions, and thus 5 prove the articles produced.

Gelatin caps are extensively employed for the purpose of forming a permanent seal for bottles and the like. In practice a cap is selected which is smaller in diameter than the 15 neck of the bottle to which it is to be applied, the cap being immersed in water for a predetermined period, during which time due to the hygroscopic nature of gelatin, the cap swells, whereupon it may be slipped over 20 the cork and the neck of the bottle and when it subsequently dries it shrinks into place around the cork and neck of the bottle, thus forming a finished and permanent seal. In order to overcome the stickiness inherent to 25 ordinary gelatin, it has been the practice in the past to subject these caps to a bath containing a certain amount of formaldehyde, or some like substance which reacts upon the gelatin and makes it insoluble, but this process of treating the caps after they have been 30 manufactured is quite laborious and technical, requiring very careful control of the proportions of the tanning agent and the temperature of the bath, in order to secure the proper degree of tanning. An under- 35 treated cap would still be sticky when it is applied and would be affected by changes in temperature and humidity, such as unusual heat, moisture or dampness after it is applied to the bottle, while a cap which received 40 too much treatment would have its tensile strength destroyed and would become very brittle and would be liable to crack or break off after it was applied.

It is therefore the object of this invention to provide a process of manufacturing these bottle caps wherein the gelatin is rendered sufficiently insoluble to withstand ordinary climatic changes of temperature and humidity, and to overcome the stickiness inherent 50 to ordinary gelatin, but at the same time not to raise the melting point of the gelatin to

such a degree where it would lose its tensile strength.

In practicing this invention a gelatin solution of the customary character and proportions is employed which usually consists of gelatin and water in the approximate proportions of 30% gelatin and 70% water, the bath or solution being maintained at a temperature of from 95° Fahrenheit to 120° Fahrenheit.

The capsule or cap is formed, in the usual or customary manner, on cooled molds or pins generally maintained at approximately 60° Fahrenheit or below.

When the proper temperature in the molds or pins has been attained, these molds are dipped, preferably a plurality at a time, into the gelatin solution or bath above referred to. The molds are then withdrawn and inverted or upturned to permit the gelatin solution which has adhered thereto, to distribute itself on the pins and to also permit the gelatin to lose its fluidity or, in other words, to change from a fluid to a plastic state. As the above method of manufacturing capsules is widely practiced and well known, and forms no part of this invention, it has only been briefly referred to.

At this state of the process, the gelatin caps contain approximately 25% or more of water. The coated molds or pins are then reversed and plunged into a tanning solution for the purpose of raising the melting point of the gelatin. This tanning solution comprises a reagent possessing an aldehydic radical, together with glycerin and water, there being a predominance of water. This tanning solution may contain in addition to the glycerin and water, either formaldehyde, hexamethylene tetramine, tannic acid, aldol, paraformaldehyde, benzaldehyde or glucose. We have found that the above ingredients mixed in substantially the following proportions give satisfactory results:

|                         | Per cent    | Per cent | Per cent      |
|-------------------------|-------------|----------|---------------|
| Formaldehyde            | 0.2 to 1.25 | 5 to 12  | 94.8 to 86.75 |
| Hexamethylene tetramine | 0.25 to 2   | 5 to 12  | 94.75 to 86   |
| Tannic acid             | 7 to 15     | 5 to 12  | 88 to 73      |
| Aldol                   | 0.25 to 2   | 5 to 12  | 94.75 to 86   |
| Paraformaldehyde        | 0.25 to 2   | 5 to 12  | 94.75 to 86   |
| Benzaldehyde            | 0.25 to 2   | 5 to 12  | 94.75 to 86   |
| Glucose                 | 15 to 30    | 1 to 10  | 84 to 60      |

The proportions of water, glycerin and the tanning agent may vary, the relative proportions being selected according to existing conditions such as the percentage of the gelatin solution used for forming the caps, type of gelatin employed in the solution and length of time the gelatin caps are left in the tanning solution, and the temperature of this tanning solution.

- 10 After being immersed in the tanning solution for a short period the molds containing the gelatin caps are removed and placed in racks or the like which are then placed in a drying room. A constant moderate temperature is maintained in the drying room as well as a moderately low degree of humidity, and the caps are allowed to remain in this drying room until their moisture content is reduced to approximately 20%, whereupon the caps will be rigid enough to strip from the molds or pins.

After the caps have been removed from the drying room the molds are run through the usual stripping machine where the caps are removed and the molds lubricated preparatory to the commencement of another cycle of operations. The caps which are stripped from the molds present an uneven edge due to the contraction of the gelatin on the molds during the drying. It is customary therefore to cut them to the proper length, whereupon they are packed for shipping or made ready for other use.

In applying to bottles or the like, gelatin caps made in accordance with this invention are immersed in cold water of a temperature preferably of 65° Fahrenheit for a period of approximately twenty minutes, whereupon they will swell or expand from approximately one and one-fourth to one and one-half times their diameter. In this condition a cap may be readily slipped over the cork and neck of the bottle and will subsequently dry, forming a smooth and permanent seal. The effect of the tanning solution upon the gelatin cap or capsule is to raise the melting point of the gelatin so that ordinarily warm temperature, or dampness and moisture will have no effect upon it. It also overcomes the stickiness inherent in a plain gelatin cap, making it easy to handle and apply to a bottle.

What we claim as our invention is:

1. In the process of manufacturing gelatinous caps, that step which consists in treating the cap externally only with one of the higher aldehydes to raise the melting point of the outer skin.
2. In the process of manufacturing gelatinous caps, that step which consists in treating the caps externally only while in a plastic state containing a large per cent of water, to raise the melting point of the outer skin.
3. In the process of manufacturing gelatinous caps, that step which consists in sub-

jecting the outer surface only of the caps while in a semi-plastic state, to the action of a tanning solution.

4. In the process of manufacturing gelatinous caps, that step which consists in subjecting the outer surface only of the caps to the action of a tanning solution including one of the higher aldehydes.

5. In the process of manufacturing gelatinous caps, that step which consists in dipping the caps while in a semi-plastic state to less than their full depth, in a bath containing a reagent possessing an aldehydic radical to treat the outer surface only.

6. In the process of manufacturing gelatinous caps, that step which consists in subjecting the caps while contained on the forming molds and while in a plastic state, to the action of a tanning solution.

7. In the process of manufacturing gelatinous caps, that step which consists of immersing the caps while in a plastic state, in a tanning bath while carried by the molds upon which the caps have been formed.

8. In the process of manufacturing gelatinous caps, those steps consisting in dipping previously cooled mold pins into a gelatin solution and immersing the caps thus formed while in a plastic state, containing 25% or more of water, in a tanning bath while they are still upon the mold pins.

9. In the process of manufacturing gelatinous caps, that step which consists in treating the outer surface only of the cap to raise the melting point of the gelatin by immersing the same to less than its full depth in a tanning solution containing benzaldehyde.

10. In the process of manufacturing gelatinous caps, that step which consists in subjecting the outer surface of the caps, while in a semi-plastic state, to the action of a tanning solution containing one of the higher aldehydes to raise the melting point of the outer skin.

11. In the process of manufacturing gelatinous caps, that step which consists in treating the cap to raise the melting point of the outer skin by dipping the same to less than its full depth in a tanning solution containing a reagent possessing an aldehydic radical, glycerine and water.

12. In the process of manufacturing gelatinous caps, that step which consists in subjecting the outer surface only of the caps, while in a plastic state, to the action of a tanning solution containing from two-tenths of one percent to thirty percent of a reagent possessing an aldehydic radical, from one to twelve percent glycerine, and from sixty to ninety-five percent water.

13. In the process of manufacturing gelatinous caps, that step which consists in subjecting the outer surface only of the caps while in a plastic state, to the action

of a tanning solution containing approximately 0.2% to 1.25% of an aldehyde, 5% to 12% of glycerine, and 94.8% to 86.75% of water.

5 14. In the process of manufacturing gelatinous caps, that step which consists in subjecting the caps, while contained on the

forming molds, to the action of an agent for rendering the skin surface thereof insoluble.

In testimony whereof we affix our signatures.

WARREN WILKIE.  
ALEXANDER D. WEBB.